

# UNITED STATES PATENT OFFICE.

ALBERT HERRMANN, OF HÖCHST-ON-THE-MAIN, GERMANY, ASSIGNOR TO THE FARBWERKE, VORMALS MEISTER, LUCIUS & BRÜNING, OF SAME PLACE.

## COLORING-MATTER.

### SPECIFICATION forming part of Letters Patent No. 412,615, dated October 8, 1889.

Application filed January 15, 1889. Serial No. 296,391. (Specimens.) Patented in Germany August 18, 1888; in Belgium September 3, 1888, No. 83,115; in France September 5, 1888, No. 192,807, and in Italy September 30, 1888, XLVII, 176.

To all whom it may concern:

Be it known that I, ALBERT HERRMANN, doctor of philosophy, a citizen of the Empire of Germany, residing at Höchst-on-the-Main, 5 in the Empire of Germany, have invented certain new and useful Improvements in Coloring-Matter, (patented in Germany August 18, 1888, F. 3,757; in Belgium September 3, 1888, No. 83,115; in France September 5, 1888, No. 10 192,807, and in Italy Vol. 47, No. 176, September 30, 1888;) and I do hereby declare the following to be a full, clear, and exact description of the invention, such as will enable others skilled in the art to which it appertains to 15 make and use the same.

My invention relates to the production of coloring-matters obtained from the etherized compounds of metaoxytetralkyldiamidotriphenyl methane



or, rather, from metamethoxy or metaethoxy tetralkyldiamido triphenyl carbinol. The sulphonic acid of these compounds dyes green-blue tints which are very fast.

In carrying out my invention I proceed as follows:

30 I. PRODUCTION OF THE ALKYL ETHERS OF METAOXYTETRALKYLDIAMIDOTRIPHENYL METHANE.

35 A. The methyl and ethyl ethers of the leuco bases



40 may be produced by condensing the tertiary aromatic amines with the corresponding alkyloxybenzaldehydes. For example, the metamethoxytetraethylidiamidotriphenyl methane is obtained by means of metaethoxybenzaldehyde (*Berichte der deutsch-45 en chemischen Gesellschaft*, 15, 2048) by heating thirty parts, by weight, of diethylaniline, twelve parts, by weight, of concentrated sulphuric acid, and 13.5 parts, by weight, of meta-

methoxybenzaldehyde three to twenty-four hours to 130° centigrade. The product of the 50 reaction is supersaturated with alkali and heated by a current of steam, and the remaining leuco base is boiled and finally dried. In a similar manner is obtained the ethoxidized leuco base by means of metaethoxybenzaldehyde



which forms at the boiling-point, which is 60 about 245° centigrade, a colorless fluid. For the production of the corresponding leuco bases are used, in the place of the diethylaniline in the same process, dimethylaniline, methylethylaniline, methylbenzylaniline, 65 ethylbenzylaniline, dimethyl-orthotoluidine, diethyl-orthotoluidine, methyl-diphenylamine, or ethyldiphenylamine.

B. The ether compounds obtained by the process just described may also be produced 70 by methylizing or ethylizing of the metaoxytetralkyldiamido triphenyl methane. These oxy leuco bases are to this effect heated for several days in a close vessel in a water-bath with three or four times their quantity of 75 alcohol, caustic soda, (one molecule,) and an excess of chloro, bromo, or iodo methyl or chloro, bromo, or iodo ethyl. Thus, for example, thirty parts, by weight, of metaoxytetraethylidiamidotriphenyl methane, twenty parts, by weight, 80 of bromo-ethyl, one hundred parts, by weight, of alcohol, and the calculated quantity of caustic soda are heated in a vessel in a water bath for forty-eight hours. Afterward the alcohol and the excess of bromo-ethyl are distilled off, 85 and the residue is boiled with water and dried. The metamethoxidized and ethoxidized tetralkyldiamidotriphenyl methanes are, when hot, semi-liquid. When cold they are brittle, pulverizable resinous bodies which show 90 but little inclination to crystallize, and in consequence of these qualities it is rather difficult to obtain them in a perfectly pure state. The one relatively most easy to be obtained in small colorless crystals is the 95 metaethoxydiethyldibenzylidiamidotriphenyl

methane. The bases dissolve readily in ether, benzol, and toluol—less readily in alcohol. Against diluted mineral acids they behave in the same way as the corresponding non-alkylized bases. Those bases deriving from dimethylaniline, diethylaniline, ethylmethylaniline, dimethyl-orthotoluidine, and diethyl-orthotoluidine are relatively stronger bases, which dissolve readily in diluted mineral acids, whereas the bases deriving from methyl and ethyl benzylaniline and from methyl and ethyl diphenylamine show scarcely any basic qualities.

15 II.—PRODUCTION OF SULPHONIC ACID OF THE METHOXIDIZED AND ETHOXIDIZED LEUCO BASES.

A. The metamethoxydized and metaethoxydized leuco bases of the generic formula



can be converted into the sulphonic acid by heating them with concentrated sulphuric acid; but, principally in consideration of the purity of the product to be obtained, it is more advantageous to use fuming sulphuric acid instead of the ordinary acid. The process is as follows:

- 30 *Example No. 1.*—Thirty parts, by weight, of metamethoxytetraethylidiamidotriphenyl methane are dissolved in one hundred and fifty parts, by weight, of fuming sulphuric acid of ten percent  $\text{SO}_3$  and the solution left standing at ordinary temperature until a sample gives with diluted ammonia a clear solution. Now the product of the reaction is poured into water and the solution converted into the calcium salt in well-known manner. 35 The calcium salt is a powder very easily soluble in alcohol and in water. In the same manner is carried out the production of the sulphonic acids respectively of their calcium salts of metaethoxytetraethylidiamidotriphenyl methane, metamethoxy and metaethoxy tetramethyldiamidotriphenyl methane, metamethoxy and metaethoxydimethyldiethylidiamidotriphenyl methane symmetric, metamethoxy and metaethoxy dimethyldiethylidiamidotriphenyl methane unsymmetric, metamethoxy and metaethoxy tetramethyldiorthotolylphenyl methane, metamethoxy and metaethoxy tetraethylidiorhodotolylphenyl methane. 45 *Example No. 2.*—Somewhat different is the process for the preparation of the sulphonic acids of those leuco bases which in the amido group still contain aromatic residues, (capable of being sulphonated,) such as benzyl or phenyl. The compounds belonging to this class are the following: metamethoxy and metaethoxy dibenzylidethyldiamidotriphenyl methane, metamethoxy and metaethoxy dibenzylidemethyldiamidotriphenyl methane, 55 metamethoxy and metaethoxy diphenyldiethylidiamidotriphenyl methane, metameth-

oxy and metaethoxy diphenyldimethyldiamidotriphenyl methane.

In the following example is described the way in which is carried out the sulphonation 70 of these leuco bases: Thirty parts, by weight, of metamethoxydibenzylidethyldiamidotriphenyl methane are dissolved in one hundred and fifty parts, by weight, of fuming sulphuric acid of twenty per cent  $\text{SO}_3$ . At ordinary temperature is formed a sulphonate acid scarcely soluble in water. Then the solution is heated for several hours to about  $70^\circ$  centigrade, until a sample dissolves easily in water with blue coloring and gives with diluted ammonia a pure blue solution having the shade of a diluted ammoniacal solution of oxide of copper. Now the product of the reaction is poured into water and converted into the calcium salt in manner well known. The sodium and calcium salts are crystalline bodies colorless in pure state and readily soluble in water and alcohol.

B. The sulphonate acid of the methoxidized and ethoxidized leuco bases can also be produced by treatment of the calcium or sodium salts of the metaoxytetralkyldiamidotriphenyl-methane sulphonic acids with methyl or ethyl halogenides.

*Example.*—Thirty parts, by weight, of the 95 calcium salt of metaoxytetraethylidiamidotriphenyl methane, twenty parts, by weight, of bromo-ethyl, and one hundred parts, by weight, of alcohol in a vessel in a water bath are heated to boiling-point for twenty to 100 twenty-four hours. The excess of bromo-ethyl and the alcohol are distilled off. To the remaining (aqueous) solution is added a small quantity of diluted sulphuric acid, and the whole is left at rest for several days, when the 105 greatest part of the leuco sulphonate acid of the ethoxidized base will have crystallized out. This is pressed off and converted into the calcium salt.

III. OXIDATION OF THE METAMETHOXIDIZED AND METAETHOXIDIZED LEUCO SULPHONIC ACIDS OF THE MALACHITE GREEN SERIES.

The calcium salts of the leuco sulphonate acids hereinbefore mentioned are converted 115 into coloring-matter by oxidation with super-oxides in presence of the calculated quantity of a mineral acid. For example, ten parts, by weight, of the calcium salt of the sulphonate acid prepared from metamethoxytetraethylidiamidotriphenyl methane are dissolved in about three hundred parts, by weight, of water. Then there are added the calculated quantities of diluted sulphuric acid and per-oxide of lead filtered off from the precipitated 120 sulphate of lead, and the blue solution of the coloring-matter is evaporated to dryness. The new coloring-matter is a copper-red powder of metallic luster, dissolving quite easily in water, giving blue color. The aqueous solu- 125 tion turns green on the addition of an excess of mineral acid. The blue color of the aque-

ous solution does not disappear on the addition of soda-lye when cold, not even when it is boiled with a solution of ammonia or soda, and it turns violet only when it is boiled with 5 soda-lye. This characteristic quality of the new coloring-matter—namely, the great resistance to the action of alkalies—is of great advantage for technical purposes and constitutes a great merit of the invention. These 10 compounds dye wool and silk in an acid bath green-blue, and excel in dyeing a level tint, in which respect the sulphonic acids of indigo are equaled. In consequence of the resistance to alkalies the tints produced are (compared to those produced with indigo-carmine) 15 very fast in washing.

IV. SULPHONATION OF METAMETHOXY AND METAETHOXY TETRALKYLDIAMIDOTRIPHENYL CARBINOL.

20 Metamethoxy and metaethoxy tetralkyldiamidotriphenyl carbinol may be converted in green-blue coloring-matter identical with the coloring-matter described in sub. III by treatment with sulphuric acid or fuming sulphuric 25 acid.

*Example.*—Ten parts, by weight, of meta-



are dissolved in one hundred parts, by weight, of monohydrate and the solution heated to 50° centigrade, until a sample dissolves in diluted 35 ammonia with blue color. The product of the reaction is converted then into the calcium or sodium salt in manner well known.

In quite the same manner analogous coloring-matter is obtained from the methyl and ethyl ethers of metaoxytetramethyldiamidotriphenyl carbinol, metaoxytetraethylidiamidotriphenyl carbinol, metaoxydimethyldiethylidiamidotriphenyl carbinol symmetric, metaoxydimethyldiethylidiamidotriphenyl carbinol unsymmetric, metaoxytetramethyldiamidodioirthotolylphenyl carbinol, metaoxytetraethylidiamidotriphenyl carbinol, metaoxydimethyldibenzylidiamidotriphenyl carbinol, metaoxydiethylidibenzylidiamidotriphenyl carbinol, metaoxydimethyldiphenylidiamidotriphenyl carbinol, and metaoxydiethylidiphenylidiamidotriphenyl carbinol.

What I claim as new, and wish to secure by Letters Patent, is—

The new fast green-blue coloring-matter obtained, as described, from the etherized compounds of metaoxytetralkyldiamidotriphenyl methane or metamethoxy or metaethoxy tetralkyldiamidotriphenyl carbinol in the form of a copper-red powder of metallic luster, easily soluble in water, and giving, when so dissolved, a blue color which remains when soda-lye is added or when boiled with a solution of ammonia or soda, changes to violet only when boiled with soda-lye, and turns green on the addition of mineral acids, as set forth.

In testimony whereof I affix my signature in presence of two witnesses.

ALBERT HERRMANN.

Witnesses:

JOSEF REVERDY,  
HEINRICH HAHN.